

## UNITED STATES PATENT OFFICE

WERNER ESPE, OF BERLIN-CHARLOTTENBURG, GERMANY, ASSIGNOR TO SIEMENS & HALSKE AKTIENGESELLSCHAFT, OF SIEMENSSTADT NEAR BERLIN, GERMANY, A GERMAN COMPANY

## METHOD FOR ACTIVATING GLOWING CATHODES OR THE LIKE

No Drawing. Application filed August 14, 1930, Serial No. 475,400, and in Germany August 19, 1929.

The invention relates to a method for activating glowing cathodes or the like by means of metals of the alkaline earth group which are formed from chemical compounds of these metals in the tube.

The oxide paste cathode which, as well known, is produced from a paste consisting of alkaline earth oxides applied to the core has the advantage of possessing an extra-  
ordinarily long life (5000 hours and more) but shows however a relatively low activity (40 milliampere per watt). This is due to the fact that during the formation process a thin layer of pure alkaline earth metal is produced on the surface of the cathode by electrolysis which displaces itself automatically from the oxide base in the course of operation. Recently one has gone over to distilling over the earth alkaline metal in metallic form on the core from an electrode whereby a complete coating of the cathode surface with alkaline earth metal and a very high activity (about 120 milliampere per watt) is obtained. In view of the fact however that the layers distilled on are very thin, the life of a cathode of this kind is considerably shorter than that of the squirted or paste cathode (about 800 to 1000 hours).

An object of this invention is the making of glowing cathodes or the like which have both the high activity of distillation cathodes and the long life of squirted or paste cathodes.

In accordance with the invention one of the alkaline earth metals, is in the well known manner, applied to the oxide paste cathode, said metal being obtained from a compound which only decomposes above the maximum temperature occurring in the tube during the formation process of the oxide paste cathode.

It was observed however that an unformed squirted cathode could not be coated with an alkaline earth metal, as on subsequent formation so much gas escaped from the cathode that the alkaline earth metal distilled on was oxidized again and its effect was thereby nullified. If, however, the oxide cathode is formed first, a high heating of the cathode and a high anode potential are neces-

sary so that the other electrode on which the alkaline earth metal source is situated glows highly. Before, however, completely terminating the formation this source must not be closed. For this reason it is not possible to use, for instance, azides of alkaline earth metals which decompose at approximately 180° centigrade.

For appropriate reasons a mixture is used, which consists of a compound of a metal of the alkaline earth group, for instance, barium oxide and aluminium or an equivalent metal, for instance, magnesium and which reacts only at temperatures over 1000° whereby metallic barium forms.

For forming a glowing cathode in accordance with the invention one may proceed in the following manner.

After evacuation, the squirted cathode is highly heated and any available carbonate decomposed into the oxide. The forming is thereupon effected with anode potential in that gradually increasing anode potentials are one after the other applied to the grid or grids and the anode, whereby simultaneously with the formation of the cathode both electrodes and the reaction mixture are raised to temperatures up to 1000° centigrade and can be well de-gassed. If the emission of the cathode has attained the desired degree the formation is terminated. After cooling of the tube has been effected, the mixture applied to the anode or situated in a special container is ignited by heating for a short time at 1100 to 1200° centigrade, in any well known manner, as by high frequency light or heat rays which are concentrated through mirrors or lenses, whereupon the reaction proceeds further automatically, until all the alkaline earth metal oxide is converted into alkaline earth metal. Owing to the speed of the reaction, the alkaline earth metal formed from the mixture only evaporates to a small extent. Therefore, it must be over-distilled to the formed oxide cathode. This is best effected by applying a potential to the heated cathode which is negative with respect to the electrode on which the reaction mixture is situated and simultaneously this electrode is heated by high frequency to about 600 to

55

60

65

70

75

80

85

90

95

100

700° C. The gradually evaporated alkaline earth metal is ionized by the electrons of the oxide cathode and the positive alkaline earth metal ions fly directly to the negative cathode and accumulate thereon to a greater extent than by ordinary temperature distillation where the major portion of the alkaline earth metal would go to the cold glass wall of the tube.

- 10 5 The method in accordance with the invention offers this advantage that the reaction temperature is substantially higher than the temperature employed for de-gassing the metal parts and forming the cathodes so that 15 the gases contained in the metal parts of the electrodes and resulting on the formation of the oxide paste cathode are removed by the pump long before the metal formed by the reaction mixture is over-distilled to the 20 formed cathode.

What is claimed is:

1. In the manufacture of electron discharge devices comprising a cathode having a coating of barium carbonate, an electrode 25 adjacent said cathode, and a mixture including barium oxide and a reducing agent upon said electrode, the method which comprises heating said carbonate to form barium oxide, applying a potential between said cathode and said electrode whereby said electrode and said mixture are out-gassed by electron bombardment, producing a reaction in said mixture to form metallic barium, applying a negative potential to said cathode and simultaneously heating said electrode to ionize said barium, and depositing said ionized barium on said cathode.
2. In the manufacture of electrode discharge devices comprising a cathode having a 40 coating of decomposable compounds of alkaline earth metal, an electrode adjacent said cathode, and a reaction mixture having a reaction temperature higher than that at which said compound is decomposable carried by said electrode, the method which comprises decomposing said compound to form the oxide of said metal on said cathode, forming said oxide coating and simultaneously out-gassing said mixture and said electrode, igniting said mixture to produce an available supply of pure alkaline earth metal, evaporating said metal, and simultaneously ionizing and accumulating said metal on the formed oxide cathode.
3. In the manufacture of electron discharge devices comprising an enclosing vessel, a cathode having a compound of an alkaline earth metal thereon, said compound being decomposable to form the oxide of said 60 metal, an electrode adjacent said cathode, and a mixture including a compound of an alkaline earth metal upon said electrode, said mixture having a reaction temperature higher than that at which said first compound is decomposable, the method which comprises

evacuating said enclosing vessel, heating said cathode to completely decompose said first compound to form the oxide of said metal, simultaneously applying a potential between said cathode and said electrode whereby said electrode and said mixture are out-gassed by electron bombardment, removing the liberated gases from said vessel, removing said potential, heating said mixture to liberate the free alkaline earth metal therefrom, applying a negative potential to said cathode, and simultaneously heating said electrode to completely transfer said metal to said oxide cathode.

In witness whereof, I hereunto subscribe my name, this 5th day of August, 1930.

WERNER ESPE.

85

90

95

100

105

110

115

120

125

130